

# UNITED STATES PATENT OFFICE.

ROBERT ABBOTT HADFIELD, OF SHEFFIELD, ENGLAND.

## MANUFACTURE OF MAGNETIC MATERIALS.

No. 851,635.

Specification of Letters Patent.

Patented April 23, 1907.

Application filed June 8, 1905. Serial No. 264,227.

*To all whom it may concern:*

Be it known that I, ROBERT ABBOTT HADFIELD, a subject of the King of Great Britain, and a resident of Sheffield, county of York, England, have invented certain new and useful Improvements in the Manufacture of Magnetic Materials, of which the following is a specification.

My invention relates to the manufacture of materials having magnetic properties, suitable for use in various electrical apparatus, such as ballast coils, transformer plates and the like.

The object of my invention is to secure a combined very low hysteresis and eddy current loss.

In former Letters Patent of the United States granted to me on December 1st, 1903, No. 745,829, and August 9th, 1904, No. 767,110, I have described the manufacture of material for the above indicated purpose by adding to iron certain proportions of silicon, aluminium or phosphorus, (either one or any two or all three of these elements) and I have also described in said patents a peculiar treatment for enhancing the desirable properties of said material or alloy. In the examples given in the said patents I have employed two of the three ingredients or additions hereinbefore mentioned, namely silicon and phosphorus, the silicon predominating very largely in relation to the phosphorus, as the amount of phosphorus used is about eleven per cent. of the amount of silicon. In carrying out further experiments for obtaining still better results, I have discovered that it is highly advantageous to increase the proportion of the addition used in conjunction with the silicon, and while silicon still forms the bulk of said addition, the percentage of the other ingredient relatively to silicon has been increased materially from the eleven per cent. previously disclosed. This will be evident from the composition of two alloys made by me in accordance with the present invention, one of which (A) contained, 3.26% silicon, .96% aluminium, .15% carbon, .1% manganese. Another alloy (B) made by me, also in accordance with the present invention, contained the elements in the following proportions: 2.47% silicon, 1.66% aluminium, .1% carbon, .03% manganese.

It will be understood that carbon and manganese are always present in materials of the class herein contemplated, and in regard to these two elements, I only wish to say that

the percentage employed should be low if the best results are desired.

The important feature of the present invention is the relative proportion of silicon and aluminium. I may state, however, that instead of aluminium I may employ phosphorus as an equivalent, or aluminium and phosphorus may be used together instead of aluminium alone. Where in the claim I have referred to aluminium, it will be understood that these equivalents are also covered. It will be seen that in Example A the proportion of aluminium to silicon is about as 1 to 3.2 or 31%. In Example B the proportion of aluminium rises to 1 to 1.5 or 66%.

The manufacture of the alloy consists simply in taking pure iron and melting it in a common crucible or electrically along with the additions named, that is silicon and aluminium (and phosphorus if such is employed). Instead of employing the crucible process I may use the decarbonized or desilicized iron produced by any steel making process such as the open hearth, the pneumatic or the electrical process, adding to such iron the desired percentage of silicon and aluminium. The molten alloy is poured into suitable ingots which, if desired, are forged or rolled into an appropriate shape. The silicon and aluminium or phosphorus may be added during the process if made in crucibles or at the end.

The material produced in accordance with my present invention so far as above described, is very valuable, since its total loss in service from hysteresis and eddy currents is very low. The material is, therefore admirably adapted for use in transformers and other electrical apparatus.

As regards the variations which may be allowable in practice in the percentage of silicon and aluminium employed, I may say that the percentage of silicon may vary from about .20 per cent. to about 5%, and the percentage of the other portion of the addition (that is, in the examples, aluminium) may vary from about .05 per cent. to about 3.75 per cent.; but so that, the proportion of aluminium or its equivalent, relatively to silicon, will be from 25% to 75%, as I have pointed out hereinbefore. This is a much higher proportion of the non-silicon addition than has been indicated in my earlier patents. Owing to the change of proportions, I have been able to secure a material improvement in the desirable electrical and magnetic

qualities of the material. The hysteresis loss of the material referred to in Example A was only .37 watts per pound for the cast material, and only .179 watts per pound for the same material rolled. For the alloy specified in Example B, the hysteresis loss was .31 watts per pound for the cast material and .214 watts per pound for the rolled material.

10 I claim as my invention:

A low hysteresis magnetic material containing iron with an addition of silicon and

aluminium; said addition amounting together to from one-fourth to eight per cent. of the iron, and the proportion of aluminium 15 amounting to from twenty-five to seventy-five per cent. of the silicon contents.

In testimony whereof, I have hereunto set my hand in the presence of two subscribing witnesses.

ROBERT ABBOTT HADFIELD.

Witnesses:

LESLIE G. WHEELER,  
EUSTACE H. BARKER.